# EUROPEAN PATENT SPECIFICATION

(11) **EP 4 341 448 B1**
(45) Date of publication and mention of the grant of the patent: **17.09.2025**
(21) Application number: 21727940.5
(22) Date of filing: 18.05.2021
(51) Int. Cl.: C21B 13/00, C21B 13/02

(54) **METHOD FOR MANUFACTURING DIRECT REDUCED IRON AND DRI MANUFACTURING EQUIPMENT**
VERFAHREN ZUR HERSTELLUNG VON DIREKT REDUZIERTEM EISEN UND DRI-HERSTELLUNGSAUSRÜSTUNG
PROCÉDÉ DE FABRICATION DE FER À RÉDUCTION DIRECTE ET ÉQUIPEMENT DE FABRICATION DE DRI

(43) Date of publication of application: 27.03.2024
(73) Proprietor: ArcelorMittal, 1160 Luxembourg (LU)
(72) Inventor: TSVIK, George, Valparaiso, IN 46385 (US); BOULANOV, Dmitri, East Chicago, IN 46312 (US); REYES RODRIGUEZ, Jon, 33400 Aviles Asturias (ES); CARRIER, Odile, 57000 Metz (FR); SALAME, Sarah, 57283 Maizieres les Metz (FR); BARROS LORENZO, José, 57283 Maizieres les Metz (FR); ANDRADE, Marcelo, East Chicago, IN 46312 (US); LU, Dennis, East Chicago, IN 46312-2939 (US)
(74) Representative: Lavoix
(86) International application number: PCT/IB2021/054256
(87) International publication number: WO 2022/243725

(56) References cited:
- RU-C1- 2 285 047
- US-A1- 2016 083 811
- US-A1- 2017 298 461
- US-B2- 9 970 071

## Description

The invention is related to a method for manufacturing Direct Reduced Iron (DRI) and to a DRI manufacturing equipment

Steel can be currently produced through two main manufacturing routes. Nowadays, most commonly used production route consists in producing pig iron in a blast furnace, by use of a reducing agent, mainly coke, to reduce iron oxides. In this method, approx. 450 to 600 kg of coke, is consumed per metric ton of pig iron; this method, both in the production of coke from coal in a coking plant and in the production of the pig iron, releases significant quantities of CO₂.

The second main route involves so-called "direct reduction methods". Among them are methods according to the brands MIDREX, FINMET, ENERGIRON/HYL, COREX, FINEX etc., in which sponge iron is produced in the form of HDRI (hot direct reduced iron), CDRI (cold direct reduced iron), or HBI (hot briquetted iron) from the direct reduction of iron oxide carriers. Sponge iron in the form of HDRI, CDRI, and HBI usually undergo further processing in electric arc furnaces. Patent documents US 2016/083811 A1 and RU 2 285 047 C1 further disclose methods for manufacturing DRI.

There are three zones in each direct reduction shaft with cold DRI discharge: Reduction zone at top, transition zone at the middle, cooling zone at the cone shape bottom. In hot discharge DRI, this bottom part is used mainly for product homogenization before discharge.

Reduction of the iron oxides occurs in the upper section of the furnace, at temperatures up to 950°C. Iron oxide ores and pellets containing around 30% by weight of Oxygen are charged to the top of a direct reduction shaft and are allowed to descend, by gravity, through a reducing gas. This reducing gas is entering the furnace from the bottom of reduction zone and flows counter-current from the charged oxidised iron. Oxygen contained in ores and pellets is removed in stepwise reduction of iron oxides in counter-current reaction between gases and oxide. Oxidant content of gas is increasing while gas is moving to the top of the furnace.

The reducing gas generally comprises hydrogen and carbon monoxide (syngas) and is obtained by the catalytic reforming of natural gas. For example, in the so-called MIDREX method, first methane is transformed into a reformer according to the following reaction to produce the syngas or reduction gas:

CH4 + CO2 ->2CO + 2H2

and the iron oxide reacts with the reduction gas, for example according to the following reactions:

3Fe203 + CO/H2 -> 2Fe3O4+CO2/H2O

Fe3O4 + CO/H2 -> 3 FeO + CO2/H2O

FeO + CO/H2 -> Fe + CO2/H20

At the end of the reduction zone the ore is metallized.

A transition section is found below the reduction section; this section is of sufficient length to separate the reduction section from the cooling section, allowing an independent control of both sections. In this section carburization of the metallized product happens. Carburization is the process of increasing the carbon content of the metallized product inside the reduction furnace through following reactions:

3Fe + CH4 → Fe3C + 2H2 (Endothermic)

3Fe + 2CO → Fe3C + CO2 (Exothermic)

3Fe + CO + H2 → Fe3C + H2O (Exothermic)

Injection of natural gas in the transition zone is using sensible heat of the metallized product in the transition zone to promote hydrocarbon cracking and carbon deposition. Due to relatively low concentration of oxidants, transition zone natural gas is more likely to crack to H₂ and Carbon than reforming to H₂ and CO. Natural gas cracking provides carbon for DRI carburization and, at the same time adds reductant (H₂) to the gas that increases the gas reducing potential.

In view of the considerable increase in the concentration of CO₂ in the atmosphere since the beginning of the last century and the subsequent greenhouse effect, it is essential to reduce emissions of CO₂ where it is produced in a large quantity, and therefore in particular during DRI manufacturing.

As explained above, it is known to use a reducing gas produced by chemically reforming a mixture of methane and top gas from the reducing furnace to produce a gas rich in hydrogen and carbon monoxide. The mixture flows through catalyst tubes where it is converted into a gas comprising hydrogen and carbon monoxide. However, such process is highly endothermic and requires the use of catalysts, which is usually Ni/Al₂O₃ that must be used at high temperatures, above 1100 K. Moreover, the catalysts are very sensible to impurities which can poison them and reduce drastically the yield of such chemical reforming process.

Based on the above, there is a need for a method of manufacturing Direct Reduced Iron that is CO₂-neutral, environmentally friendly and easy to implement, while showing a good yield.

This problem is solved by a method for manufacturing Direct Reduced Iron wherein iron ore is reduced in a DRI shaft as in appended claim 1.

The method of the invention may also comprise the following optional characteristics considered separately or according to all possible technical combinations:
- the hydrogen is mixed with said top gas before being injected in said DRI shaft,
- the reduction gas is being heated after mixing of the top gas with said hydrogen,
- the heating of the reducing gas is being done by using CO₂ neutral electricity,
- the reducing gas is being injected in the DRI shaft in its reduction section,
- the ratio of top gas to hydrogen is set from 5:1 to 1:5,
- the carbon content of the Direct Reduced Iron is set from 0.5 to 5 wt.%.

In the frame of the present invention, Direct Reduced Iron covers so-called DRI, but also hot briquetted iron (HBI), Cold Direct Reduced iron (CDRI) and Hot Direct Reduced Iron (HDRI). Such material can be later used in different processes, like, for example, processes to produce pig iron in a blast furnace or steel in a BOF or in an electric arc furnace. It can be also used as a combustible or as an electrode in a battery.

The invention is also related to a DRI manufacturing equipment including a DRI shaft and a plasma torch as disclosed in appended claim 8.

The equipment may also comprise the following optional characteristics considered separately or according to all possible technical combinations:
- a mixer can be connected on one side to the outlet of said plasma torch and to the top of the DRI shaft and, on the other side to said DRI shaft,
- heating means can be provided for the mixer, said heating means being powered by CO₂ neutral electricity,
- said mixer can be connected to the reduction section of said DRI shaft,

Other characteristics and advantages of the invention will emerge clearly from the description of it that is given below by way of an indication and which is in no way restrictive, with reference to the appended figures in which:
- Figure 1 illustrates a DRI manufacturing equipment according to the invention,
- Figure 2 illustrates a preferred embodiment of a DRI manufacturing equipment according to the invention.

Elements in the figures are illustration and may not have been drawn to scale.

Figure 1 is a schematic view of a DRI manufacturing equipment according to the invention. The DRI manufacturing equipment includes a DRI shaft 1 comprising from top to bottom an inlet for iron ore 10 that travels through the shaft by gravity, a reduction section located in the mid-part of the shaft, a cooling section located at the bottom and an outlet 12 from which the direct reduced iron is finally extracted.

On top of the shaft, the top gas exiting the DRI shaft is collected in a pipe 20 which is connected to the DRI shaft 1, creating thereby a recycling loop for such top gases to be reinjected back in the DRI shaft. The gases are travelling up to the bottom, in counter-current towards the flow of iron ore.

In a preferred embodiment, the top gas can be reinjected in the reduction section of the DRI shaft through a pipe 11.

The DRI manufacturing equipment further comprises a plasma torch 40 which is connected on one side to a methane supply 41 and, on the other side, to the DRI shaft 1 by a connecting pipe 42.

A plasma torch is a device for generating a directed flow of plasma. Thermal plasmas can be generated in plasma torches by applying electric energy to a gas. The electric energy can be direct current, alternating current, radio-frequency or other types of discharges. In a direct current torch, an electric arc is formed between the electrodes, which can be made for example of copper, tungsten, graphite or silver. The thermal plasma is formed from the input of gas, projecting outward as a plasma jet.

The most commonly used plasma types are dielectric barrier discharges, microwave and gliding arc plasmas. Dielectric barrier discharges are created by applying an electric potential difference between two electrodes, of which at least one is covered by a dielectric barrier. They typically operate at room temperature and are called cold plasmas.

Microwave and gliding arc plasmas operate at higher temperatures (typically 1000-3000 K) and are therefore called warm plasmas.

In the frame of the invention, the plasma can be created by using methane as the plasmagenic gas, allowing the non-oxidative conversion of CH₄ into hydrogen and solid carbon. Methane is transformed into an ionized gas, consisting of various chemically active species, like radicals, ions, excited atoms and molecules, and electrons. The electrons in the plasma absorb the applied electric energy and activate the molecules by excitation, ionization, and dissociation, creating the above-mentioned reactive species, which can further react to form new molecules. This allows chemical conversions to occur.

It is also possible to initiate a plasma with the use of another gas and to introduce methane in a second step in such plasma to get it transformed as described above.

The man skilled in the art knows how to control the quality of the plasma as a function of the gas pressure and the torch input power. In a preferred embodiment, the specific energy input (SEI, i.e., ratio of plasma power over gas flow rate) is ranging from 0.1 to 500 kJ I⁻¹, preferably from 100 to 400 kJ I⁻¹, allowing to reach a conversion rate of methane to hydrogen of 50 to vol 99%, preferably of 70 to vol 99%.

Plasma is very flexible and can easily be switched on/off, so it can use intermittently produced CO₂ neutral electricity from renewable sources, which cannot be stored on the grid.

CO₂ neutral electricity from renewable source is defined as energy that is collected from renewable resources, which are naturally replenished on a human timescale, including sources like sunlight, wind, rain, tides, waves, and geothermal heat.

In an embodiment, whenever hydrogen coming from the cracking of methane is not produced in a sufficient amount, due for example to the partial unavailability of electricity from renewable sources, an additional supply of hydrogen can be injected in the reduction section of the DRI shaft.

The DRI manufacturing equipment may further comprise a scrubber 2 located on the top gas outlet of the DRI shaft, before the reinjection into the shaft 1. The top gas exiting from the DRI shaft usually comprises H₂, CO, CH₄, H₂O, CO₂ and N₂ in various proportions. The top gas scrubbing operation allows removing water vapor from the rest of the stream to improve its reduction potential.

In a preferred embodiment, after scrubbing, the top gas comprises from 40 to 75 vol% of H₂, from 0 to 30 vol% of carbon monoxide CO, from 0 to 10 vol% of methane CH₄, from 0 to 25 vol% of carbon dioxide CO₂, up to 5 vol% of H₂O, the remainder being nitrogen N₂. It is preferred to have, after scrubbing, a ratio of H₂/N₂ from 1.5 to 3 in such top gas.

Once the top gas exits the scrubber 2, it can optionally be compressed and / or reheated before its reinjection in the DRI shaft through the connecting pipe 11. In a preferred embodiment, its temperature is set to a range from 700°C to 1000°C, preferably from 800 to 1000°C.

To increase the carbon content of the Direct reduced Iron, an additional source of carbon can be injected in the transition section 50 and/or in the cooling section of the shaft 1. Such additional source of carbon can be in a gaseous form and/or in a solid form and can, for example, consists of biogas and/or of bio-coal. It is also possible to use the solid carbon formed as a by-product of the plasma conversion of methane as such additional source of carbon or even as the sole source of carbon to set the carbon content of the Direct reduced Iron.

A biogas is a renewable energy source that can be obtained by the breakdown of organic matter in the absence of oxygen inside a closed system called bioreactor. Biogas can be produced from raw materials such as agricultural waste, manure, municipal waste, plant material, sewage, green waste, food waste or any biodegradable materials.

A bio-coal is a carbon-neutral fuel that can replace fossil coal in industrial processes. It is produced by pyrolysis and carbonization of biomass performed within controlled temperature and residence time conditions. Thermal conversion of biomass, which is done under oxygen-free conditions process, allows to remove volatile organic compounds and cellulose components from the feedstock and create a solid biofuel with characteristics like the ones in fossil coal.

In a preferred embodiment, the carbon content of the Direct Reduced Iron is set from 0.5 to 5 wt.%, preferably from 1 to 3 wt.% or from 2 to 3 wt.%, which allows getting a Direct Reduced Iron that can be easily handled and that keeps a good combustion potential and a good level of passivation for its future use.

The DRI manufacturing equipment may further comprise a recycling loop in the cooling section that allows extracting part of the gas present at that level to send it in a scrubber 30 and then in a compression unit 31 before reinjecting it in the shaft 1.

Figure 2 is showing a schematic DRI manufacturing equipment according to another embodiment of the invention. On top of the shaft, the top gas exiting the DRI shaft is collected in a pipe 20 which is connected to a scrubber 2, to remove water vapor from the rest of the stream, in a similar way as the equipment of Figure 1.

In a preferred embodiment, after scrubbing, the top gas comprises from 40 to 75 vol% of H₂, from 0 to 30 vol% of carbon monoxide CO, from 0 to 10 vol% of methane CH₄, from 0 to 25 vol% of carbon dioxide CO₂, up to 5 vol% of H₂O, the remainder being nitrogen N₂. It is preferred to have, after scrubbing, a ratio of H₂/N₂ from 1.5 to 3 in such top gas.

The scrubbed gas can then be sent to one of the inlet of a mixer 4 through a connecting pipe 21.

The other inlet of said mixer 4 is connected to the outlet of a plasma torch 40 to incorporate the hydrogen produced by cracking of the methane coming from the methane supply 41.

After being mixed, the reduction gas can optionally be heated through heating means provided to the mixer, such heating means being powered by CO₂ neutral electricity. In a preferred embodiment, the temperature of the reduction gas is set to a range from 700°C to 1000°C, preferably from 800 to 1000°C.

The reduction gas made of top gas and hydrogen is then sent back to the DRI shaft, preferably in its reduction section through a pipe 11.

In a preferred embodiment, the ratio of top gas to hydrogen is set from 5:1 to 1:5, preferably from 2:1 to 1:2. Such ratio is notably defined to control the respective amounts of H₂ and CO in the reduction stream. When the proportion of CO must be increased, the proportion of top gas in the reduction gas will be increased. When the proportion of H₂ must be increased, the proportion of top gas in the reduction gas will be decreased.

To increase the carbon content of the Direct reduced Iron, an additional source of carbon can be injected in the transition section 50 and/or in the cooling section. Such additional source of carbon can be in a gaseous form and/or in a solid form and can, for example, consists of biogas and/or of bio-coal. It is also possible to use the solid carbon formed as a by-product of the plasma conversion of methane as such additional source of carbon or even as the sole source of carbon to set the carbon content of the Direct reduced Iron.

In a preferred embodiment, the carbon content of the Direct Reduced Iron is set from 0.5 to 5 wt.%, preferably from 1 to 3 wt.% or from 2 to 3 wt.%, which allows getting a Direct Reduced Iron that can be easily handled and that keeps a good combustion potential for its future use.

By using the method according to the invention, Direct reduced Iron can be manufactured with the appropriate quality and yield, while remaining CO₂ neutral and taking optimal advantage of green resources like intermittent CO₂ neutral electricity from renewable sources.

## Claims

1. A method for manufacturing Direct Reduced Iron wherein iron ore is reduced in a DRI shaft by a reducing gas comprising hydrogen obtained by thermal cracking of methane inside a plasma torch, said reducing gas further comprising top gas coming from said DRI shaft, said top gas being scrubbed to remove water before being added to said reducing gas.

2. A method according to claim 1 wherein said hydrogen is mixed with said top gas before being injected in said DRI shaft.

3. A method according to claim 2 wherein such reduction gas is being heated after mixing of the top gas with said hydrogen.

4. A method according to claim 3 wherein said heating of the reducing gas is being done by using CO₂ neutral electricity produced from renewable sources chosen among sunlight, wind, rain, tides, waves, and geothermal heat.

5. A method according to anyone of the previous claims wherein said reducing gas is being injected in the DRI shaft in its reduction section.

6. A method according to anyone of the previous claims wherein the ratio of top gas to hydrogen is set from 5:1 to 1:5.

7. A method according to claim 6 wherein the carbon content of the Direct Reduced Iron is set from 0.5 to 5 wt.%.

8. A DRI manufacturing equipment including a DRI shaft (1) and a plasma torch (40), wherein said plasma torch (40) is connected on one side to a methane supply (41) and, on the other side, to said DRI shaft (1), said DRI shaft (1) being provided with a recycling loop allowing to inject its top gas back in said DRI shaft (1), the equipment further comprising a scrubber (2) connected to the top gas outlet of the DRI shaft (1) to remove water from the top gas.

9. A DRI equipment according to claim 8, further including a mixer (4) connected on one side to the outlet of said plasma torch (40) and to the top of the DRI shaft (1) and, on the other side to said DRI shaft (1).

10. A DRI equipment according to claim 9, further including heating means for the mixer (4), said heating means being powered by CO₂ neutral electricity produced from renewable sources chosen among sunlight, wind, rain, tides, waves, and geothermal heat.

11. A DRI equipment according to claims 9 or 10, wherein said mixer (4) is connected to the reduction section of said DRI shaft (1).

## Patentansprüche

1. Verfahren zum Herstellen von direkt reduziertem Eisen, bei dem Eisenerz in einem DRI-Schacht durch ein Reduktionsgas reduziert wird, das Wasserstoff umfasst, der durch thermisches Cracken von Methan in einem Plasmabrenner erlangt wird, wobei das Reduktionsgas ferner Gichtgas umfasst, das aus dem DRI-Schacht stammt, wobei das Gichtgas gewaschen wird, um Wasser zu entfernen, bevor es zu dem Reduktionsgas hinzugefügt wird.

2. Verfahren nach Anspruch 1, wobei der Wasserstoff mit dem Gichtgas gemischt wird, bevor er in den DRI-Schacht eingeleitet wird.

3. Verfahren nach Anspruch 2, wobei das Reduktionsgas nach Mischen des Gichtgases mit dem Wasserstoff erhitzt wird.

4. Verfahren nach Anspruch 3, wobei das Erhitzen des Reduktionsgases unter Verwendung von CO₂-neutralem Strom erfolgt, der aus erneuerbaren Quellen erzeugt wird, die ausgewählt sind aus Sonnenlicht, Wind, Regen, Gezeiten, Wellen und Erdwärme.

5. Verfahren nach einem der vorherigen Ansprüche, wobei das Reduktionsgas in den DRI-Schacht in seinen Reduktionsabschnitt eingeleitet wird.

6. Verfahren nach einem der vorherigen Ansprüche, wobei das Verhältnis von Gichtgas zu Wasserstoff auf 5:1 bis 1:5 eingestellt wird.

7. Verfahren nach Anspruch 6, wobei der Kohlenstoffgehalt des direkt reduzierten Eisens auf 0,5 bis 5 Gewichts-% eingestellt wird.

8. DRI-Herstellungsanlage, die einen DRI-Schacht (1) und einen Plasmabrenner (40) beinhaltet, wobei der Plasmabrenner (40) auf der einen Seite mit einer Methanzufuhr (41) und auf der anderen Seite mit dem DRI-Schacht (1) verbunden ist, wobei der DRI-Schacht (1) mit einer Rückführschleife versehen ist, die es ermöglicht, sein Gichtgas zurück in den DRI-Schacht (1) zu leiten, wobei die Anlage ferner einen Wäscher (2) umfasst, der mit dem oberen Gasauslass des DRI-Schachts (1) verbunden ist, um Wasser aus dem Gichtgas zu entfernen.

9. DRI-Anlage nach Anspruch 8, ferner umfassend einen Mischer (4), der auf einer Seite mit dem Auslass des Plasmabrenners (40) und mit dem oberen Ende des DRI-Schachts (1) und auf der anderen Seite mit dem DRI-Schacht (1) verbunden ist.

10. DRI-Anlage nach Anspruch 9, ferner umfassend eine Heizeinrichtung für den Mischer (4), wobei die Heizeinrichtung mit CO₂-neutralem Strom betrieben wird, der aus erneuerbaren Quellen erzeugt wird, die ausgewählt sind aus Sonnenlicht, Wind, Regen, Gezeiten, Wellen und Erdwärme.

11. DRI-Anlage nach Anspruch 9 oder 10, wobei der Mischer (4) mit dem Untersetzungsabschnitt des DRI-Schachts (1) verbunden ist.

## Revendications

1. Procédé de fabrication de minerai de fer préréduit dans lequel le minerai de fer est réduit dans un puits DRI par un gaz réducteur comprenant de l'hydrogène obtenu par craquage thermique du méthane à l'intérieur d'une torche à plasma, ledit gaz réducteur comprenant en outre du gaz de tête provenant dudit puits DRI, ledit gaz de tête étant nettoyé pour éliminer l'eau avant d'être ajouté audit gaz réducteur.

2. Procédé selon la revendication 1, dans lequel ledit hydrogène est mélangé au gaz de tête avant d'être injecté dans le puits DRI.

3. Procédé selon la revendication 2, dans lequel le gaz réducteur est chauffé après le mélange du gaz de tête avec ledit hydrogène.

4. Procédé selon la revendication 3, dans lequel le chauffage du gaz réducteur est effectué en utilisant de l'électricité neutre en CO₂ produite à partir de sources renouvelables choisies parmi la lumière du soleil, le vent, la pluie, les marées, les vagues et la chaleur géothermique.

5. Procédé selon l'une quelconque des revendications précédentes, dans lequel le gaz réducteur est injecté dans le puits DRI dans sa section de réduction.

6. Procédé selon l'une quelconque des revendications précédentes, dans lequel le rapport entre le gaz de tête et l'hydrogène est compris entre 5:1 et 1:5.

7. Procédé selon la revendication 6, dans lequel la teneur en carbone du minerai de fer préréduit est comprise entre 0,5 et 5 % en poids.

8. Équipement de fabrication de DRI comprenant un puits DRI (1) et une torche à plasma (40), dans lequel ladite torche à plasma (40) est connectée d'un côté à une alimentation en méthane (41) et, de l'autre côté, au puits DRI (1), ledit puits DRI (1) étant pourvu d'une boucle de recyclage permettant de réinjecter son gaz de tête dans le puits DRI (1), l'équipement comprenant en outre un épurateur (2) connecté à la sortie du gaz de tête du puits DRI (1) afin d'éliminer l'eau du gaz de tête.

9. Équipement DRI selon la revendication 8, comprenant en outre un mélangeur (4) connecté d'un côté à la sortie de ladite torche à plasma (40) et au sommet du puits DRI (1) et, de l'autre côté, au puits DRI (1).

10. Équipement DRI selon la revendication 9, comprenant en outre des moyens de chauffage pour le mélangeur (4), lesdits moyens de chauffage étant alimentés par de l'électricité neutre en CO₂ produite à partir de sources renouvelables choisies parmi la lumière du soleil, le vent, la pluie, les marées, les vagues et la chaleur géothermique.

11. Équipement DRI selon les revendications 9 ou 10, dans lequel ledit mélangeur (4) est relié à la section de réduction du puits DRI (1).
